

## UNITED STATES PATENT OFFICE

2,139,515

## ALLOYS FOR ADDITION TO IRON AND STEEL

George L. Norris, Scarsdale, N. Y., assignor to  
Vanadium Corporation of America, Bridgeville,  
Pa., a corporation of Delaware

No Drawing. Application April 25, 1938, Serial  
No. 204,190

3 Claims. (Cl. 75—58)

This invention relates to an alloy containing silicon, titanium, zirconium, and iron, and especially to an alloy suitable for addition to molten iron and steel for the purpose of obtaining a more sound, dense and clean metal when such steel or iron solidifies.

The present application is a continuation-in-part of my copending application, Serial No. 128,230, filed February 27, 1937.

10 The use of ferro-silicon, ferro-titanium, ferro-zirconium, iron-silicon-zirconium, and iron-silicon-titanium for the purpose of scavenging molten steel and iron is very well-known and is more or less generally employed in steel and iron manufacturing practice. Their use, however, involves very marked deficiencies so that, while they free the molten metal of impurities, such as iron oxide and iron nitride by chemically reacting with these compounds, the products: iron silicates, titanium cyanonitrides, and zirconium cyanonitrides, remain entrapped in the metal, thereby imparting to it several objectionable qualities. The amount of non-metallics remaining entrapped in the metal is not always the same. Therefore, iron and steel alloys are obtained which have varying physical qualities, such as ductility, although of the same chemical composition.

20 I have discovered that the combination of all three elements—silicon, titanium and zirconium—with iron, in proper proportions, produces an alloy which when added to molten iron and steel reacts with gaseous and other impurities in the molten metals to form reaction products which more readily coagulate and separate from the molten iron or steel. My alloy is readily soluble in molten iron or steel and is more effective and economical than alloys containing only one or two of the elements silicon, titanium and zirconium in combination with iron.

25 My alloy not only acts as a scavenger in molten iron and steel, i. e., removes the various impurities in the molten metal but also serves to control the grain size of the treated product.

30 35 While my alloy is composed of silicon, titanium, zirconium and iron and is substantially free from carbon, there may be present small percentages of other elements incidental to the method of production or in the raw materials used. For example, the chemical composition of one melt of this alloy which may be considered typical in respect to the presence of the other metals, is:

|           | Per cent |
|-----------|----------|
| Silicon   | 40.28    |
| Titanium  | 10.62    |
| Zirconium | 10.49    |
| Carbon    | 0.07     |
| Aluminum  | 1.53     |
| Manganese | 0.76     |
| Iron      | Balance  |

This alloy is substantially free from carbon, but the carbon content may vary up to a maximum of about 1.0% or even up to 4.0%, depending upon the method of manufacture and intended use. In many cases, I prefer to have the carbon below 0.15%.

10 This improved composition of my present invention consists of an alloy with a minimum amount of carbon, so as to be substantially free from carbon, and contains about 25% to 60% silicon, preferably about 25% to 45% silicon, about 5% to 20% or 25% titanium, and about 5% to 20% or 25% zirconium. In no case, however, does the sum of the silicon, titanium and zirconium exceed 85%. The percentage of silicon is at least equal to or greater than the percentage of either the titanium or zirconium. The remainder of the alloy is principally iron, although usual impurities or small amounts of other alloying elements may be present.

15 20 25 While I have described my alloy in its preferred composition, it is to be understood that the invention is not so limited, but may be otherwise embodied within the scope of the following claims.

I claim:

30 35 40 1. An alloy for addition to iron and steel, containing about 25% to 60% silicon, about 5% to 25% titanium, about 5% to 25% zirconium, the sum of the silicon, titanium and zirconium not exceeding 85%, and not over about 4.0% carbon, the remainder being principally iron.

2. An alloy for addition to iron and steel, containing about 25% to 60% silicon, about 5% to 25% titanium, about 5% to 25% zirconium, the sum of the silicon, titanium and zirconium not exceeding 85%, and not over about 1.0% carbon, the remainder being principally iron.

3. An alloy for addition to iron and steel, containing about 25% to 45% silicon, about 5% to 20% titanium, about 5% to 20% zirconium, and not over about 0.15% carbon, the remainder being principally iron.

45 50 GEORGE L. NORRIS.